

# UNITED STATES PATENT OFFICE.

JOEL CLARKSON DECKER, OF LABORATORY, PENNSYLVANIA.

## OIL FOR GENERAL PAINTING.

SPECIFICATION forming part of Letters Patent No. 454,035, dated June 16, 1891.

Application filed September 24, 1890. Serial No. 366,012. (No specimens.)

*To all whom it may concern:*

Be it known that I, JOEL CLARKSON DECKER, a citizen of the United States, residing at Laboratory, in the county of Washington and 5 State of Pennsylvania, have invented a new and useful Oil for General Painting, of which the following is a specification.

The composition employed in my invention consists of the following ingredients, combined in the proportions stated, viz: crude petroleum, one gallon; yellow beeswax, one-fourth to one-half pound; pulverized resin, one-half pound; sulphate of zinc, one-eighth to one-fourth pound; sugar (acetate) of lead, 10 one-eighth to one-fourth pound; litharge, one-fourth to one-half pound; linseed-oil, one-half to one pint. These ingredients are to be thoroughly mingled by agitation while in a state of ebullition.

20 The process of preparing the above composition is as follows: First dissolve the sugar of lead and sulphate of zinc in warm water; then add this solution to the petroleum; then heat this second solution (the oil, lead, and

zinc) to 212° Fahrenheit, and stir the compound so as to thoroughly mix the ingredients. Now add the beeswax and resin, and when these are thoroughly dissolved add the litharge and linseed-oil. Stir well and let it cool.

The above composite oil gives a good vehicle for painter's use in mixing their various paints. It is non-volatile, inodorous, and has about the specific gravity of good linseed-oil. It is also a good water-proof oil, and is 35 possessed of excellent antiseptic and preservative powers.

What I claim, and desire to secure by Letters Patent of the United States, is—

A paint vehicle or oil for painters' use, composed of crude petroleum, yellow beeswax, pulverized resin, sulphate of zinc, acetate of lead, litharge, and linseed-oil, in substantially the proportions herein set forth.

JOEL CLARKSON DECKER.

Witnesses:

JNO. C. BANE,

JNO. H. HOCHAL.